

May 24, 1938.

F. M. CRAPO

2,118,758

PROCESS OF MAKING ZINC COATED FERROUS WIRE

Filed Oct. 25, 1935



Fig. 2.



Carbon Content: Per Cent

Inventor  
Frederick M. Crapo

By

Jehly - Tracy

Attorneys

## UNITED STATES PATENT OFFICE

2,118,758

PROCESS OF MAKING ZINC-COATED  
FERROUS WIREFrederick M. Crapo, Muncie, Ind., assignor to  
Indiana Steel & Wire Company, Muncie, Ind.,  
a corporation of IndianaApplication October 25, 1935, Serial No. 46,782  
In Canada June 5, 1934

10 Claims. (Cl. 91—70.3)

It is the object of my invention to produce zinc-coated ferrous wire which is of relatively low carbon content but which has both high tensile strength and good zinc adhesion.

5 Ferrous wires with good zinc adhesion, even with very low carbon content, have been made. Among such wires are those shown in the Crapo Patent No. 1,501,887, granted July 15, 1924; in the Crapo Patent No. 1,552,041, granted September 1, 1925; and in the Crapo and Baylis Patent No. 1,545,305, granted July 7, 1925.

10 My co-pending application Serial No. 705,831, filed January 8, 1934, now Patent No. 2,019,445, granted October 29, 1935, is directed to an electric transmission line embodying a ferrous wire of relatively low carbon content but of high tensile strength. My present application is directed to the process of making and zinc-coating such a wire, and more especially the wire made 20 use of in that application.

15 While other wires with both good zinc adhesion and high tensile strength are known, in general they have been rather high in carbon; whereas my present invention is directed to the 25 combining of good zinc adhesion and high tensile strength in a ferrous wire of relatively low carbon content—in any event less than 0.50% carbon, and desirably less than 0.25% carbon—and with the manganese desirably below 0.50%, and 30 below 0.30% when the carbon exceeds 0.25%.

25 In carrying out my invention, I treat such a ferrous wire at elevated temperature, preferably in a molten-salt bath of suitable character, to produce on the surface of the wire by chemical 35 change a permeative addition of material of the class consisting of carbon and nitrogen and phosphorus, and thereafter quench the wire from a temperature at least as high as the  $A_{c1}$  critical temperature, and desirably from a temperature 40 at least as high as the  $A_{c3}$  critical temperature, in a liquid medium which has a temperature below the melting point of lead; and then I coat the wire with zinc, desirably by a hot-galvanizing process in which I also partially draw the temperature 45 of the wire by heat treatment after the quenching.

30 Various types of apparatus may be used for carrying out the process of my invention. In the accompanying drawing I show one such apparatus diagrammatically. In that drawing, Fig. 1 is a diagrammatic view of a heating and quenching apparatus, with a subsequent tempering apparatus and a subsequent wire-drawing apparatus, either or both of which may be used if desired, 50 and in addition an apparatus for a preliminary

salt treatment and an apparatus for a subsequent zinc-coating treatment; and Fig. 2 is a diagram showing the contents of carbon and manganese in the carbon-steel wire, the area in solid-line cross-hatching indicating the preferred area, 5 and the area in broken-line cross-hatching indicating the permissive area.

The apparatus shown diagrammatically in Fig. 1 is for carrying out my invention on ferrous wire 10 of the character shown in Fig. 2. That is, 10 it is a carbon-steel wire in which the carbon is below 0.50%, and desirably below 0.25%; and the manganese is also fairly low, in any case below 1.0% and desirably below 0.50%, and below 0.30% when the carbon exceeds 0.25%. Silicon, 15 phosphorus, and sulphur may be present in the amounts common in carbon steels. These carbon steels may be copper-bearing steels.

This carbon-steel wire 10, which may already have been subjected to some or all of any desired 20 wire-drawing before reaching the apparatus shown in Fig. 1, is ordinarily passed first through a pickling or other cleaning bath 11. Then it is passed through a heating device, which is preferably in the form of a molten-lead bath 12; 25 from which it emerges through a band or rim 13 of the type shown in the Crapo and Baylis Patent No. 1,545,305 already referred to. Within the band or rim 13 is a bath of molten salt 14, which is of such character, as by containing cyanide or 30 cyanamid, that it produces by chemical change such a permeative addition on the surface of the wire 10 that adhesion of a subsequently applied zinc coating is improved, as set forth in my prior Patent No. 1,501,887 already referred to. As the wire 10 passes through the molten material of the lead bath 12, and/or of the salt bath 14, it is heated toward or to the 35 desired temperature from which it is later to be quenched; so that less additional heating or even no additional heating is required before subsequent quenching. That is, the heating within the baths 12 and 14 may in some cases be sufficient to raise the temperature of the wire 10 to 40 the desired value from which it is to be quenched. Ordinarily, however, the wire 10 on leaving the molten-salt bath 14 passes into a heating furnace 15, in which its temperature is further elevated to the desired temperature from which 45 quenching is to be done; so that the temperatures of the molten lead and of the molten salt may be lower than when these baths are required to do all the heating prior to quenching.

The temperature to which the wire is thus 50 raised by the baths 12 and 14, and by the fur- 55

nace 15 if it is used, is at least as high as the  $A_{c1}$  or lowermost critical temperature, and desirably as high as the  $A_{c3}$  or uppermost critical temperature. As is well known, these critical temperatures vary with the composition of the ferrous material.

The heating furnace 15 is conveniently but not necessarily of the muffle type. The atmosphere within it may be of any suitable character. Such atmosphere may be one which in itself tends to produce by chemical change in the surface of the ferrous wire a permeative addition which tends to promote the adhesion of a subsequently applied zinc coating, such as ammonia gas (of the Crapo Patent No. 1,552,041 already referred to) or phosphine gas; in which case the bath 14 of molten cyanide or cyanamid may be omitted.

From the heating furnace 15, the wire 10 passes immediately into a quenching bath 16, in which while still at or above the critical temperature it is immediately immersed in a liquid quenching medium. Such quenching medium is one which in any case has a temperature below the melting point of lead, and in many instances desirably has a temperature at or below the boiling point of water. This quenching from at or above the critical temperature to this relatively low temperature carries the temperature of the carbon-steel wire very rapidly downward through the critical temperature range, so that the wire then has high tensile strength.

The liquid quenching medium may be water, or any desired aqueous solution, especially for ferrous wires in the lower range of carbon contents, say below 0.25%. Oil, or other suitable organic liquid, may also be used for the quenching medium. So may a low-melting salt or mixture of salts, or low-melting metal or alloy, melting in any case below the melting point of lead.

After the wire 10 leaves the quenching bath 16, a partial drawing of its temper is often desirable, especially in wire of the higher carbon contents (within the range of my invention), when the quenching has been in a quenching medium of the water type, and/or when the subsequent zinc-coating is by a cold process. This may be obtained by passing the wire through a suitable tempering furnace 17. When such a tempering furnace is employed, it raises the temperature of the wire to the temperature necessary for drawing the temper to the desired extent.

The temperature of the tempering furnace 17 may vary with the composition of the wire, usually being higher as the carbon content is greater; with the suddenness and extent of the chilling produced by the quenching, usually being higher as such chilling has been more drastic; with the character of subsequent treatments, such as whether the subsequent zinc-coating is by the hot-dip process or by a cold process such as electro-plating; and with the tensile strength and other characteristics desired in the wire.

After leaving the quenching bath 16 (and the tempering furnace 17 if it is used), the wire 10 is suitably zinc-coated. Preparatory to this it is usually passed through any of the well-known preliminary treatments, such as a pickling bath 18 and a fluxing bath 19. After these preliminary treatments, the wire 10 passes to the zinc-coating bath 20.

The zinc-coating bath 20 may be of any desired character, to deposit zinc either hot or cold—as by hot-dipping or by electro-deposition. Desirably it is a hot-galvanizing tank, in which

case the zinc is maintained molten by suitable heating means 21 shown diagrammatically below the zinc-coating bath 20. By having the zinc-coating bath 20 a hot-galvanizing bath, it is of especial advantage to use the bath of molten salts 14, to promote adhesion of the zinc to the ferrous wire. Moreover, when the coating bath 20 is a hot-galvanizing bath it inherently involves a heat treatment of the wire 10 passing through it. That heat treatment partially draws the temper of the wire from the greater hardness produced in the quenching bath 16, so that it is then commonly not necessary or desirable to use a tempering furnace 17 in addition; but my invention does not preclude the use of both on the same wire, for the extent of the tempering may be varied as desired in my invention.

From the zinc-coating bath 20, the wire 10 passes to a take-up reel 22, by which power is applied to the wire for pulling it through the apparatus.

If desired, one or more wire-drawing dies 23 may be provided to act on the wire after it has been quenched and/or after it has been zinc-coated. The drawing produced by these dies 25 supplements the increase in tensile strength obtained by the quenching.

By the process which has been described, a zinc-coated ferrous wire of relatively low carbon content may be obtained which has both a tensile strength which is high and a zinc adhesion which is superior, as compared with ordinary ferrous wires of corresponding carbon content.

The apparatus shown in the drawing is merely illustrative, and may be varied in many respects. My invention does not depend on any particular apparatus. Instead, it is directed broadly to the process as defined in the appended claims.

I claim as my invention:

1. The process of treating a steel wire which contains less than 0.50% carbon, and which contains less than 0.30% manganese when the carbon exceeds 0.25%, which consists in subjecting said wire to an elevated temperature under conditions which produce on its surface by chemical change a permeative addition of material of the class consisting of carbon and nitrogen and phosphorus, thereafter quenching the wire from a temperature at least as high as the  $A_{c1}$  critical temperature in a liquid medium having a temperature below the melting point of lead, and then zinc-coating it by the hot-dip process.

2. The process of treating a steel wire which contains less than 0.50% carbon, and which contains less than 0.30% manganese when the carbon exceeds 0.25%, which consists in subjecting said wire to an elevated temperature under conditions which produce on its surface by chemical change a permeative addition of material of the class consisting of carbon and nitrogen and phosphorus, thereafter quenching the wire from a temperature at least as high as the  $A_{c3}$  critical temperature in a liquid medium having a temperature below the melting point of lead, and then zinc-coating it by the hot-dip process.

3. The process of treating a steel wire which contains less than 0.50% carbon, and which contains less than 0.30% manganese when the carbon exceeds 0.25%, which consists in passing said wire through a molten-salt bath which by chemical change produces on the surface of the wire a permeative addition of material of the class consisting of carbon and nitrogen, thereafter quenching the wire from a temperature at least as high as the  $A_{c1}$  critical temperature in a liquid medium

having a temperature below the melting point of lead, and then zinc-coating it by the hot-dip process.

4. The process of treating a steel wire which contains less than 0.50% carbon, and which contains less than 0.30% manganese when the carbon exceeds 0.25%, which consists in passing said wire through a molten-salt bath which by chemical change produces on the surface of the wire a permeative addition of material of the class consisting of carbon and nitrogen, thereafter quenching the wire from a temperature at least as high as the  $Ac_1$  critical temperature in a liquid medium having a temperature below the melting point of lead, and then zinc-coating it by the hot-dip process.

5. The process of treating a steel wire which contains less than 0.25% carbon, which consists in subjecting said wire to an elevated temperature under conditions which produce on its surface by chemical change a permeative addition of material of the class consisting of carbon and nitrogen and phosphorus, thereafter quenching the wire from a temperature at least as high as the  $Ac_1$  critical temperature in a liquid medium having a temperature below the melting point of lead, and then zinc-coating it by the hot-dip process.

6. The process of treating a steel wire which contains less than 0.25% carbon, which consists in subjecting said wire to an elevated temperature under conditions which produce on its surface by chemical change a permeative addition of material of the class consisting of carbon and nitrogen and phosphorus, thereafter quenching the wire from a temperature at least as high as the  $Ac_1$  critical temperature in a liquid medium having a temperature below the melting point of lead, and then zinc-coating it by the hot-dip process.

7. The process of treating a steel wire which contains less than 0.25% carbon and less than 0.50% manganese, which consists in subjecting said wire to an elevated temperature under conditions which produce on its surface by chemical change a permeative addition of material of the class consisting of carbon

and nitrogen and phosphorus, thereafter quenching the wire from a temperature at least as high as the  $Ac_1$  critical temperature in a liquid medium having a temperature below the melting point of lead, and then zinc-coating it by the hot-dip process.

8. The process of treating a steel wire which contains less than 0.25% carbon and less than 0.50% manganese, which consists in subjecting said wire to an elevated temperature under conditions which produce on its surface by chemical change a permeative addition of material of the class consisting of carbon and nitrogen and phosphorus, thereafter quenching the wire from a temperature at least as high as the  $Ac_1$  critical temperature in a liquid medium having a temperature below the melting point of lead, and then zinc-coating it by the hot-dip process.

9. The process of treating a steel wire which contains between 0.25% and 0.50% carbon and not in excess of 0.30% manganese, which consists in subjecting said wire to an elevated temperature under conditions which produce on its surface by chemical change a permeative addition of material of the class consisting of carbon and nitrogen and phosphorus, thereafter quenching the wire from a temperature at least as high as the  $Ac_1$  critical temperature in a liquid medium having a temperature below the melting point of lead, and then zinc-coating it by the hot-dip process.

10. The process of treating a steel wire which contains between 0.25% and 0.50% carbon and not in excess of 0.30% manganese, which consists in subjecting said wire to an elevated temperature under conditions which produce on its surface by chemical change a permeative addition of material of the class consisting of carbon and nitrogen and phosphorus, thereafter quenching the wire from a temperature at least as high as the  $Ac_1$  critical temperature in a liquid medium having a temperature below the melting point of lead, and then zinc-coating it by the hot-dip process.

FREDERICK M. CRAPO. 45